

June 25, 1946.

J. A. CLARK

2,402,653

PROCESS AND APPARATUS FOR SIZING YARNS

Filed Nov. 17, 1943



INVENTOR.  
James Andrew Clark

BY Frank A. Steinbauer

ATTORNEY.

## UNITED STATES PATENT OFFICE

2,402,653

PROCESS AND APPARATUS FOR SIZING  
YARNS

James Andrew Clark, White Plains, N. Y., assignor to Sylvania Industrial Corporation, Fredericksburg, Va., a corporation of Virginia

Application November 17, 1943, Serial No. 510,608

3 Claims. (Cl. 28—28)

1

The invention relates in general to a process and apparatus for sizing warp yarns and to correlated improvements designed to enhance the properties of the warp yarns in weaving.

It is known to size warp yarns, prior to weaving, with an aqueous solution of water-soluble colloids, such as starch, gum, dextrine, gelatine, in order to facilitate the weaving of such yarns. In the prior practice, however, the use of these water-soluble substances for sizing the warp yarns has been attended by certain disadvantages. The process has been slow and hence expensive because of the high viscosity, slow penetration and low drying ratio of the solutions used. Moreover, yarns sized with water-soluble colloids show a pronounced decrease in stiffness after the first laundering; must be de-sized prior to dyeing, mercerizing or bleaching, which in itself decreases the yarn resistance; and have in any case a low resistance to abrasion, which causes the nap to be raised during weaving. It is also necessary to carry out the weaving of such prior yarns in an atmosphere of relatively high humidity, which tends to corrode the metal parts of the loom.

To obviate these difficulties and disadvantages, it is now proposed to size the warp yarns prior to weaving with an alkali-soluble water-insoluble cellulosic colloid. This novel size presents many advantages over the use of water-soluble substances heretofore used, in fact its use obviates all the difficulties mentioned above, but alkali-soluble water-insoluble cellulosic colloids possess the property of being inherently tacky, causing the yarns to adhere to each other during the sizing operation, and this raises a new difficulty which it is the object of the present invention to overcome.

It is the general object of the present invention to provide a process and apparatus for slashing warp yarns in a rapid and economical manner.

It is a specific object of the invention to provide a process for permanently sizing a multiplicity of warp yarns in a continuous manner.

It is another specific object of the invention to provide an apparatus for slashing warp yarns which is adapted to be used for sizing the yarns with a tacky size.

Other objects of the invention will in part be obvious and will in part appear hereinafter.

According to the present invention, there is provided a process of sizing a multiplicity of warp yarns with a tacky composition prior to weaving while avoiding the adhesion of adjacent yarns to each other. More particularly, the invention relates to a process for collectively sizing a multiplicity of warp yarns while arranged in the form

5 of a weftless web with an alkaline dispersion of an alkali-soluble water-insoluble cellulosic colloid, separately coagulating said colloid on the individual warp yarns, whereby the nap on the yarns is permanently laid and the twist stabilized, and drying the yarns.

10 The apparatus of the invention comprises, in combination, means to treat warp yarns in the form of a weftless web, with a liquid sizing composition, in particular an aqueous dispersion of a water-insoluble coagulable colloid, means to separate the yarns, means for coagulating the colloid on the yarns while so separated, and means for drying the yarns. The apparatus preferably includes means for separating the yarns before and after coagulating the colloid thereon whereby the yarns do not adhere to each other in passing through the subsequent treating devices.

15 The invention accordingly comprises a process having the steps and the relation of steps one to another, and an apparatus having the elements and relation of elements, one to another, as set forth in the following detailed description and the scope of the application of which will be indicated in the claims.

20 The present process is applicable for slashing singles yarns and plied yarns of all types, in particular, warp yarns comprising cotton, ramie, jute, flax, casein, and rayon, also fibres formed of cellulose derivatives and synthetic resins, or mixtures of these fibres, and whether carded or combed, or made of continuous filaments or staple fibres.

25 The process and apparatus of the present invention may be used with any warp sizing composition but in particular with tacky compositions such, for example, as an aqueous dispersion, preferably an alkaline dispersion of alkali-soluble water-insoluble cellulosic colloid. For the cellulosic colloid there may be employed the alkali-soluble water-insoluble cellulosic ethers as a class, such for example as alkyl-cellulose ether, hydroxy-alkyl cellulose ether, carboxy-alkyl cellulose ether, and the like; also, the alkali-soluble 30 water-insoluble cellulose materials per se as a class, such, for example, as cellulose dissolved in any of its known solvents, such as an alkali solution of 5% to 10% concentration, alkaline solutions of zincates, and stannates, or strong organic bases such as aralkyl ammonium hydroxides; also alkali-soluble water-insoluble degraded cellulose 35 such, for example, as the degraded cellulose solutions disclosed in the co-pending U. S. application Serial No. 427,389 filed January 19, 1942, and the 40 degraded cellulose solutions disclosed in U. S. Pat-

ent No. 2,289,085, and in British Patent No. 507,138; also starch, rosin, resin, rubber latex and other sizes may be used.

Among the cellulose ether solutions, there is preferred an alkali-soluble water-insoluble hydroxy-ethyl cellulose ether dissolved in an aqueous alkali solution, and among the cellulosic solutions, there is preferred a degraded cellulose dissolved in an aqueous alkaline zincate solution as disclosed in U. S. Patent No. 2,289,085.

The cellulosic colloid may be coagulated from its alkaline dispersion by means of any of the known coagulants for viscose, such, for example, as acids, acid salts, salts and heat, also by the action of hot water.

The alkaline dispersion of the cellulose colloid is preferably applied to the yarn while the dispersion has a low viscosity. It is characteristic of the degraded cellulose solutions above disclosed that their alkaline dispersions have very low viscosities. However, alkali solutions of the cellulose ethers may be made of low viscosity either (a) by degrading the cellulose ether before or after its manufacture by the use of heat alone or by heating with acids, alkalies, or oxidizing agents; or (b) the viscosity of the alkaline solutions may be lowered by adding to the solution an oxidizing agent; or by heating the aqueous alkaline solution of the cellulose ether during application to the yarn to a temperature at which it shows a pronounced drop in viscosity such, for example, as a temperature between 140° and 160° F.

The cellulosic content of the alkaline dispersion may be varied over a wide range, but usually if the dispersion contains from 3% to 8%, preferably about 6% by weight of the solution of the cellulosic colloid, a satisfactory warp sizing will be obtained. The quantity of alkali, which is normally a strong alkali such as sodium hydroxide, potassium hydroxide or aralkyl-ammonium hydroxide, may be varied according to the amount required to completely and uniformly disperse the cellulosic colloid, which amount is usually between 5% and 10% by weight of the solution.

To the dispersion there may also be added a wetting agent such, for example, as a sulfated fatty alcohol, a sulfonated fatty acid, and the like. Likewise, there may be added to the sizing composition, pigments or dyestuffs which are stable in alkali. Since the sizing agent will not be removed after weaving nor during laundering, the pigments or dyestuffs will serve to permanently color the yarns, a feature which cannot be achieved by the use of conventional starch or other water-soluble colloids. The coagulated water-insoluble colloid serves to permanently bind the pigments or dyestuffs to the yarns.

For a more complete understanding of the nature and objects of the present invention, reference should be had to the accompanying drawing in which there is illustrated one embodiment of the apparatus of the invention for permanently sizing warp yarns.

Fig. 1 is a diagrammatical representation in side elevation of one embodiment of the yarn sizing apparatus of the invention;

Fig. 2 is a longitudinal view, partly in section, of one of the yarn separating rollers utilized in the apparatus shown in Fig. 3, and

Fig. 3 is a diagrammatical representation in side elevation of a second embodiment of the yarn sizing apparatus of the invention.

Referring to Fig. 1, the warp yarns 10 are unwound from the beam 11 and passed into the

sizing composition held in the first box 12 of a four-box slasher. The box 12 is provided with a jacket 13 and, in the space so provided, hot water is introduced through the pipe 14 and withdrawn through the pipe 15. The remaining boxes 16, 17 and 18 of the slasher are substantially identical in construction, and each is provided with a submerged roller 19, and a pair of pressure rollers 20 positioned above each box respectively, so that the excess liquid carried by the yarns is caused to flow back into the respective box. The pressure rollers 21 and 22 at the exit of the box 12 are of special construction. It has been found that to avoid flattening the yarns and to produce an even distribution of the size thereon, one or both of the rollers 21 and 22 is provided with a very rough surface, for example, by wrapping the roller with a very rough fabric such, for example, as burlap. The top roller 21 will normally be the wrapped roller and the bottom roller 22 will be a roller provided with a soft resilient surface such as rubber. The rollers are provided with a means (not shown) for subjecting the yarn to substantial pressure as it passes between the rollers.

From the nip of the rollers 21 and 22, the sized warp yarns 10 are separated by a leash or splitter rod 23, and the size, e. g. a cellulosic colloid, coagulated as the yarn passes through a liquid coagulant contained in box 16. After coagulation the yarns are again separated by a leash or splitter rod 23. The yarns are washed, e. g. with hot water contained in box 17 and may be subjected to a second washing e. g. with dilute alkali in the box 18. After this treatment, the sized yarns are dried by suitable means as by passing them over and under the heated drying cans 24 and 25, and the dried yarns are then wound upon the beam 26, which may be a split beam. To prevent overlapping of the yarns one upon the other, there may be provided, at suitable points in the course of travel, combs or reeds 27 of conventional design, such reeds being shown in the figure at points where the yarns leave the box 17, the box 18, and before and after they pass over the drying cans.

It is important and highly desirable that the warp yarns be separated, as by passing alternate yarns over and under the leash or splitter rods 23 and 23', before and after coagulation of the size, e. g. the cellulosic colloid, since the coagulation of the size while the yarns are in contact tends to cause adjacent yarns to adhere to each other.

By way of illustrating, but not by way of limiting the invention, there will be given the following example:

Combed or carded cotton warp yarns, intended for use in twills or drills for military uniforms, are sized by passing the yarns through a sizing composition comprising 6% alkali-soluble water-insoluble cellulose ether (initial viscosity of 2 compared to glycerin), 8% sodium hydroxide, and the remainder water. To this solution is added 0.2% of ammonium persulfate which reduces the relative viscosity of the composition by oxidation to between 0.5 and 0.1. The sizing composition is placed in the box 12 of the apparatus shown in the drawing and the composition heated to a temperature of 150° F. The warp yarns are passed successively through the hot composition contained in box 12, then through the pressure rollers 21 and 22, separated by the leash rod 23, and then passed into the box 16 containing a 5% aqueous solution of sulphuric acid as a coagulant. The excess coagulant is

squeezed out by means of the pressure rollers 20, the yarn separated by the rod 23, and then washed in water contained in the box 17 heated to 140° F. Finally, the yarns are subjected in the box 18 to washing with an aqueous solution of 5% ammonia, and the washed yarns are then dried on the cans 24 and 25.

In Fig. 3 there is shown a second embodiment of the apparatus of the invention, in which the multiplicity of the yarns 10 are unwound from the beam 11 and passed over tension rolls 8 and 9 and then into a slasher having boxes 12, 16, 17 and 18 similar to those of the apparatus shown in Fig. 1. Likewise, the pressure rollers 21 and 22 at the exit of box 12 have the same surface as the rollers 21 and 22 in the apparatus of Fig. 1. The apparatus shown in Fig. 3 differs from that shown in Fig. 1 in that the yarn separating means are rotatable rollers. Such means are provided for saturating the yarns with the cellulosic colloid while the yarns are separated from each other at least over a part of their path through the bath. For example, by providing in the box 12 two submerged rotatable rollers 1 and 2, alternate yarns pass under the roller 1 and the other yarns pass under roller 2, all the yarns passing through the nip of the rolls 21 and 22 as in the apparatus of Fig. 1. Further, in Fig. 3, the sized yarns 10 are maintained in a separated condition during coagulation by passing alternate yarns under the submerged roller 3 of box 16 and the intervening yarns first over a roller 4 and then under a submerged roller 5, all the yarns passing under a common roller 30 and through the nip of the rollers 20. Thus, adjacent yarns are not in contact and are separated as they pass into the coagulant contained in the box 16. The yarns pass from the box 16 into the box 17 where they are washed. It has been found that if the yarns are separated during coagulation of the size, it is not essential that they be separated during washing, although box 17 may likewise be provided with separating rolls as in the box 16 of Fig. 1 or splitter rods like the rods 23 shown above in box 17 in Fig. 1. After washing in box 17, the yarns are subjected to a second washing in the box 18. Sprays 29 of washing fluid may be positioned to wash the yarns as they pass between the rollers 20. Thereafter the yarns are dried in a suitable manner, for example by the means shown in the apparatus of Fig. 1.

It has been found that to facilitate the proper feeding of the yarns through the nip of the rolls 21, 22 and the squeeze rolls 20, it is advisable to align the yarns just before they contact these rolls. This may be done, for example, by positioning grooved rollers 31 above each bath and adjacent the rolls 22 and 20 so that the individual yarns 10 are caused to pass into the grooves 32 of the roller 31 before the yarns contact the rolls 22 and 20. A suitable grooved roller is shown in Fig. 2, it being understood that the number of the grooves may be varied as needed to take care of all the yarns that have to pass over the roller 31.

The process and apparatus of the invention may be readily adapted for coloring some or all of the warp yarns, for purposes of identification, decoration, and the like. For example, when it is desired to color some, but not all, of the warp yarns, a second size box 12a may be positioned in front of the box 12 as shown in Fig. 3. Yarns 10a are then led from a second beam 11a through a colored sizing composition contained in the box 12a, alternate yarns passing under the roller,

1a and the other yarns 2a, all of the yarns 10a being passed through a common padder comprising the rolls 21a and 22a.

The colored yarns are then passed by means of a roller 33 over the padder comprising rolls 21 and 22 and are then separated so that alternate yarns pass over the roller 4a and then under the roller 8 while the other yarns pass over the roller 4b and then under the roller 9.

Simultaneously, the yarns 10 from the beam 11 are being treated in the bath 12 and passed through the nip of the rollers 21 and 22 and the rollers 3 and 5, respectively, so that the colored and uncolored yarns come together and pass under the common roll 30 after which the yarns are treated collectively in the remaining boxes 17 and 18.

It is to be understood that the sizing composition in the box 12 may be colorless or colored a different color than the sizing composition in the box 12a. Since the colored yarns do not contact each other until the size has been coagulated in the box 16, while the yarns are maintained separate from each other, there will be no bleeding of the colors from one set of yarns to another. After coagulation, the differently colored yarns pass together side by side through the remaining treatments but there is no bleeding because the size has already been coagulated. It is to be understood that when dyestuffs are employed for coloring the yarns, the leuco compound of the dye may be employed in the size boxes 12 or 12a and the developer for the dye may be incorporated in the box 18 in compatible admixture with the coagulating agent. Suitable dyestuffs which can be added to alkaline solutions of cellulosic colloids in a two-step treatment as just described are disclosed and claimed in my prior U. S. Patent No. 2,259,796.

The present process and apparatus embody many advantages over prior and conventional means of slashing warp yarns. In the first place, the present invention provides means for treating a multiplicity of the yarns while arranged as a weftless web without permitting the yarns to stick together when sized because the yarns are separated in passing into the coagulating bath and preferably also while being sized. By this means, the yarns are individually impregnated and/or coated with the size and individually treated with coagulants and, if desired, individually washed, whereupon the nap fibres are laid, the twist stabilized and the yarns given a relatively smooth surface and suitably stiffened to facilitate weaving. Finally, means have been provided for the first time of coloring some or all of the warp yarns without having the color bleed upon the adjacent colored or differently colored yarns.

It is also to be understood that the following claims are intended to cover all of the generic and specific features of the invention herein described, and all statements of the scope of the invention which, as a matter of language, might be said to fall therebetween.

Having described my invention, what I claim as new and desire to secure by Letters Patent is:

1. In an apparatus for sizing warp yarns with a coagulable tacky composition, the combination of, means to treat a multiplicity of warp yarns with said tacky composition, a pair of pressure rollers for subjecting said yarns to pressure while the yarns are wet with said composition, a grooved roller positioned prior to and adjacent to said pressure rollers for leading the yarns in parallel

separate relation between said pressure rollers, means to pass said yarns through a coagulant for said composition, and means to maintain said yarns in a separated state while they are passing through said coagulant.

2. In an apparatus for sizing warp yarns with a coagulable tacky composition, the combination of, a plurality of vats adapted to contain different sizing compositions, means for passing some of the warp yarns through one of said vats, means for passing alternate warp yarns through the other vat, a pair of pressure rollers for subjecting each of said sets of yarns to pressure while wet with said composition, a grooved roller positioned prior to and adjacent said pressure rollers, means

10 15

to pass all of said yarns through a coagulant of said compositions, and means to separate the yarns while they are passing through said coagulant.

3. In a process for sizing warp yarns with a coagulable tacky composition, the steps comprising treating alternate yarns with one sizing composition and treating the other yarns with a different sizing composition, separately subjecting both sets of yarns to pressure while said yarns are maintained in a separated state and passing all of said yarns through a common coagulant while maintaining said yarns in a separated state while passing through said coagulant.

JAMES ANDREW CLARK.